

## UNITED STATES PATENT OFFICE

HEINRICH BRUNNER, OF BASEL, SWITZERLAND, ASSIGNOR TO THE FIRM "CHEMICAL WORKS FORMERLY SANDOZ", OF BASEL, SWITZERLAND

## DYEING OF CHAMOIS-LEATHER

No Drawing. Application filed December 24, 1928, Serial No. 328,317, and in Germany January 5, 1928.

Up to recently shades on chamois-leather, which are fast to washing, could only be obtained with dye-wood extracts of which the scale of shades is a very limited one. Besides the different grey and brown shades no comparatively fast dyeings could be obtained; more particularly the fastness to soaping was not satisfactory.

Recently various trials have been undertaken with the object to obtain soap proof and otherwise fast shades with sulphur dyes. The dyeing with sulphur dyes requires alkalis of such a concentration that an injurious effect on the skin cannot be avoided.

The chamois-leather dyed with vat and sulphur dyes is, with regard to its characteristic properties, such as touch and elasticity, so considerably altered that these methods did not find any acceptance.

Other processes are known, according to which the injurious action of the alkalis has been reduced by the addition of protective colloids (glucose, gelatine, soaps) or substances of similar action such as glycerine, formaldehyde, sulphite cellulose waste, where the formaldehyde especially acts in a hardening manner. By the use of these methods, the above mentioned characteristic properties of chamois-leather could not be maintained, especially when the leather has been dyed with vat and sulphur dyes.

It has now been found that by a pretreatment of chamois-leather with appropriate inorganic oxidizing agents as well as with similarly acting organic substances, the dyeing operation can be so considerably accelerated that the dyeing is finished before the alkalis have been able to act in an injurious manner on the leather. As inorganic oxidizing agents the following enter into consideration: hydrogen peroxide, perborates or halogens, and among organic substances the halogen acylamids ("chloramines") may be useful. Chamois-leather dyed in this manner conserves its characteristic properties such as touch and elasticity, and the dyeings thus obtained are level and fast to washing and soaping. The alkali sulphide necessary for dyeing with sulphur dyes is evidently partially oxidized on the leather and the dye-

stuff is fixed. It is not necessary to expose the skins to air in order to oxidize the dye-stuffs.

To finish the dyeing and for obtaining bright shades it may be advantageous to subject the dyeings to an aftertreatment in an oxidizing bath, containing, for instance, acid reacting inorganic oxidizing agents, such as alkali bichromates or another acid or neutral metal salt solution of oxidizing properties of which an acidulated alkali metal nitrite solution is of special value.

This new manner of dyeing chamois-leather represents a technical progress.

The following examples illustrate the improved process.

*Example 1.* 100 g. of chamois-leather are thoroughly washed, if necessary with some alkali or soap. Thereupon the leather is milled in a solution of 5 g. of alkali metal perborate in 3 litres of water during an hour and subsequently squeezed out and shortly rinsed.

Afterwards 6 g. of thional green B (Colour Index No. 1006) and the necessary quantity of sodium sulphide are dissolved in 2 litres of water and the leather dyed in a closed dyeing apparatus. After 20-30 minutes the dyebath is exhausted. The leather is then squeezed out and afterwards subjected to an aftertreatment by handling it in a watery solution containing 2 g. of sodium bichromate and 5 g. of concentrated acetic acid. Thereupon the leather is rinsed and soaped.

*Example 2.* 100 g. of chamois-leather are thoroughly cleaned and afterwards treated with a mixture of 25 ccm. of a clear hypochlorite of lime solution in 3 litres of water, whereupon the hypochlorite reaction disappears rather quickly from the solution.

At the same time the smell cannot be observed anymore. The leather is afterwards hydroextracted and can then be brought into the dyebath containing 6 g. of thional indon blue R, (Colour Index No. 959) and 6 g. of anhydrous sodium sulphide. When the bath is exhausted, the leather is pressed out, hydroextracted and aftertreated with a bichromate solution as indicated in Example 1.

*Example 3.* 100 g. of thoroughly cleaned

chamois-leather are handled in 3 litres of water containing 2 g. of the sodium salt of p-toluene sulphonic chloramide, whereupon it is possible to regulate the gradual setting 5 free of chlorine by a slow addition of diluted or weak acids. After a sufficient treatment with a watery solution of 2 g. of acetic acid, the leather is pressed, shortly rinsed and dyed in a bath containing 15 g. of thional black T 10 (Colour Index No. 978) and 18 g. of anhydrous sodium sulphide. After half an hour of dyeing no increase in the depth of the tone is obtained, whereupon the after-oxidation with bichromate and acetic acid, 15 according to Example 1, is effected. Subsequently the leather is rinsed and redyed in the same bath. After a second oxidation with bichromate the leather is washed and soaped.

20 *Example 4.* 100 g. of chamois-leather are thoroughly washed and afterwards treated with a mixture of 15 ccm. of a hypochlorite of lime solution of 4° Bé. in 1 liter of water during 15 minutes. Thereupon the leather 25 is duly pressed out. Then 5 g. of ciba red R (Colour Index No. 1229), 10 g. of concentrated sodium sulphide and 3 g. of hydro-sulfite are dissolved in 250 ccm. of water of 40° C. and the leather dyed at a temperature of 30-40° C. in a closed apparatus.

After 20 minutes of dyeing the leather is shortly rinsed in running water. Thereupon the after oxidation with bichromate and sulphuric acid is effected. Subsequently the 35 leather is rinsed and treated with some soap and yolk in the usual manner.

In the foregoing example any other vat dyestuffs such as ciba red G (Colour Index No. 1226), ciba violet B (Colour Index No. 40 1222) and so on may be used with similar effects.

What I claim is:

1. A process for dyeing chamois-leather, comprising the steps of treating chamois- 45 leather with compounds yielding chlorine and dyeing same immediately after this treatment with dyestuffs being reduced in the dyebath.

2. A process for dyeing chamois-leather, 50 comprising the steps of treating chamois-leather with compounds yielding chlorine and dyeing same immediately after this treatment with sulphur dyes.

3. A process for dyeing chamois-leather, 55 comprising the steps of treating chamois-leather with an aqueous solution of hypochlorite of lime and dyeing same immediately after this treatment with sulphur dyes.

In witness whereof I have hereunto signed  
60 my name this 12th day of December, 1928.

HEINRICH BRUNNER.